

March 19, 1929.

J. A. HOLLADAY

1,706,293

CONCENTRATION OF COPPER ORES

Filed Aug. 11, 1926

Explosibility  
of  
Acetylene-Nitrogen-Air Mixtures



Inventor:

James A. Holladay,  
By <sup>33.3</sup> Townsend & Brickenden,  
Attorneys.

Patented Mar. 19, 1929.

1,706,293

# UNITED STATES PATENT OFFICE.

JAMES A. HOLLADAY, OF DOUGLASTON, NEW YORK, ASSIGNOR TO UNION CARBIDE SALES COMPANY, A CORPORATION OF WEST VIRGINIA.

## CONCENTRATION OF COPPER ORES.

Application filed August 11, 1926. Serial No. 128,677.

The invention relates to the concentration of copper ores by froth flotation, and in particular to the treatment of oxidized copper minerals, such as malachite, cuprite and chrysocolla, to render them amenable to such flotation. It is known that only the sulphide ores of copper are satisfactorily floatable, and it has been proposed to treat the oxidized ores with acetylene to increase their floatability. The invention comprises improvements in the process last referred to.

The acetylene can be applied in a variety of ways, and either simultaneously with the grinding of the ore or after grinding is completed. Previously prepared gaseous acetylene may be injected into the pulp of ore and water, or merely brought into contact with the surface of the liquid, or a solution of acetylene in water or other solvent may be mixed with the ore or pulp, or calcium carbide may be added to the pulp whereupon the water present will of course decompose the carbide and produce acetylene.

As an incident to several of the desirable methods of applying the acetylene, the ore is subjected to the oxidizing action of atmospheric air. The air may be initially present in the water used or it may be taken up by the water when the latter is agitated in the presence of air, as where the ore is ground while the acetylene is being applied to it. My experiments indicate that the action of air is undesirable, and that it interferes with the effect sought to be brought about by the acetylene, at least when air has unrestricted access to the pulp. Furthermore, explosive mixtures of air and acetylene may be formed in and around the grinding mills and other apparatus, and the presence of such explosive mixtures is an undesirable hazard.

The invention consists in preventing or diminishing contact of the ground ore with oxygen by displacing or diluting with an inert gas the air which might otherwise act on the ore. Flue gases, or more or less pure nitrogen or carbon dioxide, are mentioned as examples of inert gases suitable for this purpose.

The inert gas is preferably admixed with the acetylene in such proportions that non-explosive mixtures are produced. Where the atmosphere in contact with the ore contains sufficient inert gas to render it non-explosive, the concentration of oxygen pres-

ent will in general be insufficient to interfere seriously with the action of the acetylene on the ore.

In the annexed drawing I have indicated on a triaxial diagram those mixtures of acetylene, air, and nitrogen which are non-explosive. It will be understood that the explosibility of a gas mixture cannot be stated with precision, inasmuch as it is largely influenced by the shape and size of the vessel containing the mixture, and by the character of the means used for ignition. An intense or "fat" spark will ignite many mixtures which can not be ignited by a less energetic spark of the same length. In the experiments on which the diagram is based, the gas mixtures were saturated with water vapor at 25° C., and were subjected to the action of a rather thin spark 1/4 inch in length while held in a spherical bulb of approximately 3 inches diameter, the spark gap being at the center. All ignitable mixtures were classified as explosive, even though combustion proceeded quietly under the test conditions. The tests were arranged with a view to simulating conditions which might arise in the treatment of ores with acetylene.

It will be apparent that displacement of air by inert gas in accordance with the invention may be effected in many different ways, depending on the manner in which the acetylene is applied. Procedure which has given good results is to flow the pulp into a ball mill arranged to be closed gas-tight or nearly so; pass nitrogen into the mill until the oxygen concentration is sufficiently diminished; add calcium carbide while substantially preventing access of air; grind the charge; and then discharge the mill.

I claim:

The process of preparing oxidized copper minerals for froth flotation which comprises suspending the finely ground mineral in water as a pulp, treating the mineral particles with acetylene, and preventing aeration of the pulp during the process by displacing air in contact therewith by a non-combustible, inert gas, whereby the action of the acetylene on the mineral particles is intensified.

In testimony whereof, I affix my signature.

JAMES A. HOLLADAY.